

# United States Patent

Schlunke et al.

[15] 3,656,953

[45] Apr. 18, 1972

[54] **SILVER DYESTUFF BLEACHING  
PROCESS USING QUINOXALINE  
CATALYST**

[72] Inventors: **Hans-Peter Schlunke, Marly-le-Petit; Karl Roneo, Riehen, both of Switzerland**

[73] Assignee: **Ciba-Geigy AG, Basel, Switzerland**

[22] Filed: **Mar. 3, 1970**

[21] Appl. No.: **16,207**

[30] **Foreign Application Priority Data**

Mar. 13, 1969 Switzerland ..... 3820/69

[52] **U.S. Cl.** ..... 96/53, 96/20, 96/73,

96/99

[51] **Int. Cl.** ..... G03c 7/00

[58] **Field of Search** ..... 96/53, 99, 73

[56] **References Cited**

## UNITED STATES PATENTS

3,429,705 2/1969 Piller et al..... 96/53

|           |         |                     |       |
|-----------|---------|---------------------|-------|
| 2,669,517 | 2/1954  | Mueller .....       | 96/53 |
| 2,270,118 | 1/1942  | Gaspar .....        | 96/99 |
| 3,443,949 | 5/1969  | Oetiker et al. .... | 96/53 |
| 3,443,947 | 5/1969  | Mory et al. ....    | 96/53 |
| 3,278,303 | 10/1966 | Meyer et al. ....   | 96/53 |

*Primary Examiner*—J. Travis Brown

*Attorney*—Harry Goldsmith, Joseph G. Kolodny and Mario A. Monaco

[57] **ABSTRACT**

A process for the manufacture of color photographic images according to the dyestuff bleaching process is provided. In this process the dyestuff bleaching is carried out in the presence of a dyestuff bleaching catalyst which is a quinoxaline substituted in the 2- and 3-positions by alkyl or aryl groups and also the benzene nucleus may be further substituted. These quinoxalines possess a good activity and effect an advantageous gradation.

**16 Claims, No Drawings**

SILVER DYESTUFF BLEACHING PROCESS USING  
QUINOXALINE CATALYST

The subject of the present invention is the use of quinoxalines of formula

(1)



wherein  $A_1'$  and  $A_2'$  each denote an alkyl residue with at most 5, preferably 1, carbon atoms or an at most bicyclic aryl residue, preferably a benzene residue,  $D'$  denotes a residue of formula  $-\text{CN}$ ,  $-\text{O}-\text{R}$ ,  $-\text{COO}-\text{R}_1$  or



, wherein  $R$  represents an alkyl residue with at most five carbon atoms and  $R_1$  and  $R_2$  each represent a hydrogen atom or an alkyl residue with at most five carbon atoms, and  $E$  denotes a hydrogen or halogen atom, an alkyl or alkoxy group with at most five carbon atoms, a nitro group or optionally further-substituted amino group, as colour bleaching catalysts in the silver dyestuff bleaching process.

Advantageously, quinoxalines of formula

(2)



are used, wherein  $A_1$  and  $A_2$  each denote a methyl or phenyl residue,  $E$  has the significance indicated and  $D$  denotes a residue of formula  $-\text{O}-\text{R}$ ,  $-\text{COO}-\text{R}_1$  or



, wherein  $R$  represents an alkyl residue with at most five carbon atoms and  $R_1$  and  $R_2$  each represent a hydrogen atom or an alkyl group with at most five carbon atoms.

Preferably, quinoxalines of formula

(3)



and especially of formula

(4)



are used, wherein  $A_2$ ,  $D$  and  $E$  have the indicated significance.

Quinoxalines which are very suitable correspond to the formula

(5)



wherein  $D_1$  denotes an alkoxy group with one to four carbon atoms and  $E_1$  a hydrogen or halogen atom, an alkyl or alkoxy group with at most 5 carbon atoms, a nitro, amino or alkylamino group with at most four carbon atoms or an

75

and especially those of formula

acylamino group, and  $A_1$  and  $A_2$  have the indicated significance.

Amongst these quinoxalines, those of formula

5

(6)



10

and above all of formula

(7)



15

wherein  $D_2$  denotes a methoxy or ethoxy group and  $E_2$  denotes a chlorine atom or a methyl, methoxy, nitro, amino, methylamino or acylamino group, with acyl representing the residue of an alkanecarboxylic acid with one to five carbon atoms or of an optionally further-substituted benzenecarboxylic acid or heterocyclic carboxylic acid, and  $E_1$ ,  $A_1$  and  $A_2$  have the indicated significance, are of special interest.

Preferred acyl residues in  $E_2$  are residues of alkanecarboxylic acids, for example residues of acetic, propionic or butyric acid or benzenecarboxylic acid residues, for example benzoic acid, toluic acid, chlorobenzoic acid, bromobenzoic acid, nitrobenzoic acid, salicylic acid, methoxybenzoic acid or aminobenzoic acid residues. Possible residues of heterocyclic carboxylic acids are for example residues of pyridinecarboxylic, furanecarboxylic and thiophene-carboxylic acids.

Amongst the quinoxalines of formula (7), quinoxalines of

(8)



40

and especially those of formula

(9)



45

wherein  $E_3$  denotes a methoxy, methylamino or amino group and  $D_2$  and  $A_2$  have the indicated significance, again occupy a preferred position.

Other quinoxalines of formula (5), with which favourable results are achieved, correspond to the formula

(10)



60

wherein  $E_1$ ,  $A_1$  and  $A_2$  have the indicated significance. Of these quinoxalines, those of formula

(11)



70

and especially those of formula

(12)



wherein  $A_2$ ,  $E_2$  and  $E_3$  have the indicated significance, are preferred.

Here the use of quinoxalines of formula

(13)



wherein  $E_3$  has the indicated significance, has proved particularly advantageous.

Quinoxalines which are monosubstituted in the benzene ring preferably correspond to the formula

(14)



wherein  $D_3$  represents a residue of formula  $-\text{CN}$ ,  $-\text{COO}-R_1$  or



, wherein  $R_1$  and  $R_2$  each denote an alkyl residue with at most five carbon atoms or a hydrogen atom, and  $A_1$  and  $A_2$  have the indicated significance.

Here, quinoxalines of formula

(15)



are above all very suitable, wherein  $D_4$  represents a residue of formula  $-\text{COO}-R_1$ , wherein  $R_1$  denotes an alkyl residue with at most five carbon atoms or a hydrogen atom, and  $A_1$  and  $A_2$  have the indicated significance.

Amongst the quinoxalines of formula (15), those of formula

(16)



wherein  $A_2$  has the indicated significance, and especially those of formula

(17)



are of great interest.

Instead of the free carboxylic acids, it is also possible to employ the corresponding salts, such as for example alkali, ammonium, or alkaline earth salts or other derivatives which can easily be converted into free carboxylic acid under the dyestuff bleaching conditions.

The residues  $D'$  or  $D$  and  $E$  in formulae (1) to (4), or the residues  $D_1$ ,  $D_2$ ,  $E_1$ ,  $E_2$  and  $E_3$  in formulae (5) to (13), can be in the 5-, 6-, 7- or 8-position of the quinoxaline ring system. Preferably, however, the  $E$  and  $D$  residues are in the o-position or p-position to one another.

The quinoxalines of formula (1) can be used as dyestuff bleaching catalysts in a processing bath, preferably the dyestuff bleaching bath, and/or in a layer of the photographic material.

5 They can be employed either alone or in the presence of other customary dyestuff bleaching catalysts. It is also possible to employ different quinoxalines of formula (1) simultaneously in the dyestuff bleaching bath. Finally, the quinoxalines of formula (1) can also be employed together with other measures which promote bleaching, such as for example together with an irradiation of the dyestuff bleaching bath or bubbling a gas through the dyestuff bleaching bath or adding organic solvents to the dyestuff bleaching bath.

15 The quinoxalines of formula (1) can thus be incorporated into a layer which is free of dyestuff which can be bleached image-wise. The multi-layer material can thus for example possess an additional gelatine layer containing only the catalyst, this layer being located directly on the layer support or between two colour layers. In the latter case the layer containing the catalyst also acts as a dividing layer. Furthermore, the catalyst can also be incorporated into colloidal silver or into filter layers containing an organic yellow filter dyestuff or into coating layers. These filter layers, like the layers with the 20 image dyestuffs, appropriately contain gelatine as the layer colloid.

25 The quinoxalines of formula (1) can however also be directly incorporated into a layer containing an image dyestuff. In other respects, the multi-layer material can display the usual composition. Using the photographic materials of the composition indicated, dyestuff-photographic images can be produced in the usual manner which is in itself known.

The dyestuff bleaching catalysts of formula (1) can however, as already mentioned, also for example be added to the 30 colour bleaching bath, where they then exert their action directly. They can also be added to a prior treatment bath, for example to the developer, a hardening bath, a stopping bath or a special bath before the silver dyestuff bleaching bath. Here a certain part of the amount of catalyst employed is taken up by

40 the photographic layer material and retained until it can then become effective in the dyestuff bleaching bath. The amount of catalyst to be used can vary within wide limits depending on the type of use. In general, it suffices for a strong effect to add 0.001 to 0.1 g of catalyst per 1 litre of a dyestuff bleaching 45 bath of the usual composition which contains a silver complex-forming agent such as for example an alkali bromide or iodide or thiourea and optionally an oxidation protection agent such as for example sodium hypophosphite, and a strong 50 organic or inorganic acid, such as for example benzenesulphonic acid, hydrochloric acid, sulphuric acid, phosphoric acid or sodium bisulphite for reaching the requisite pH-value.

Further subjects of the invention are, accordingly, also a 55 photographic light-sensitive material for the silver dyestuff bleaching process which contains a quinoxaline of formula (1) as a dyestuff bleaching catalyst in at least one layer on a support, and photographic processing baths, especially dyestuff bleaching baths, characterised in that they contain at least one 60 quinoxaline of formula (1) as a dyestuff bleaching catalyst.

A further subject of the invention is then a process for the manufacture of color-photographic images according to the silver dyestuff bleaching process on materials which on a support contain at least one silver halide emulsion layer with a dye-stuff which can be bleached image-wise, by exposure, development of the silver image and dyestuff bleaching, characterised in that the dyestuff bleaching is carried out in the presence of at least one quinoxaline of formula (1) as the colour bleaching catalyst.

70 The hitherto known compounds used as dyestuff bleaching catalysts in the silver colour bleaching process exert very different effects on azo dyestuffs of different constitution. Whilst they are very effective with one class of azo dyestuffs, they can display only a slight bleaching-promoting effect towards 75 another class. There is thus a need for compounds which by



If the appropriate o-phenylenediamine is accessible simply and in adequate purity, it is condensed directly, or in the form of its hydrochloride, with the desired diketone in a suitable solvent under nitrogen. When using the hydrochloride it is advisable to add a corresponding amount of sodium or potassium acetate to neutralise the HCl liberated.

In order to synthesise 2,3-asymmetric compounds, the  $\alpha$ -diketone is replaced by  $\alpha$ -bromopropiophenone. The 1,2-dihydroquinoxaline thus formed is then oxidised with the Na salt of m-nitrobenzenesulphonic acid in the presence of aqueous NaOH to give the quinoxaline.

The redox potentials are determined by means of polarography in the customary manner which is in itself known. A mixture of dimethylformamide-2 N sulphuric acid in the ratio of 1 : 1 serves as the solvent in all cases. The potential is measured against an Ag/AgCl electrode of known potential and is then recalculated to the potential against a normal hydrogen electrode. Whilst in some cases two single-electron transitions, characterised in that two polarographic waves occur, are observed, only a single polarographic wave is observed in other cases, and this then corresponds to the mean redox potential.

The melting points and analytical results of all quinoxalines of formula (1) which were manufactured are summarized in Table I.

A. 6-Ethoxy-2,3-dimethylquinoxaline ml 10% 3.55  
13.71100% ml

9.1 g (50 mmols) of 4-ethoxy-2-niranoline are dissolved in 200 ml. of ethanol, mixed with 1 g of 10 percent strength palladium-charcoal catalyst and hydrogenated at room temperature under normal pressure. The reaction temperature rises to 41° C over the course of 10 minutes and to 53° C over the course of the following 15 minutes, with 3.55 l of hydrogen being consumed. The temperature then gradually drops to 26° C. The total hydrogen consumption amounts to 3.7 l = 100 percent of theory. The catalyst is filtered off in a closed apparatus under nitrogen and the dark red filtrate is mixed with 4.3 g (50 mmols) of diacetetyl in a stream of nitrogen. The reaction mixture is then heated for 10 minutes under nitrogen to the reflux temperature. After cooling, 300 ml of water are added and the whole is cooled to 0° C. The 6-ethoxy-2,3-dimethylquinoxaline which has precipitated is filtered off, washed with a little water and dried at 60° C in vacuo. Yield : 7.1 g (70% of theory) of light yellow crystals of the compound A. The thin layer chromatogram with chloroform: ethyl acetate = 7:3 as the migrating agent shows a single substance with an R<sub>f</sub>-value of 0.57. The infrared spectrum and the nuclear resonance spectrum are in agreement with the expected structure.

B. 2-Methyl-3-phenyl-6,7-dimethoxyquinoxaline

2.3 g (10 mmols) of 4,5-dinitroveratrole are dissolved in 170 ml of absolute alcohol, mixed with 0.2 g of 10% strength palladium charcoal and hydrogenated under normal pressure at room temperature. The temperature rises to 38° C over the course of 15 minutes and then again drops to 27° C over the course of a further hour, with 1.47 l (= 100% of theory) of hydrogen being taken up. The catalyst is filtered off under nitrogen in a closed vessel, with the colourless filtrate being directly charged onto 0.98 g (12 mmols) of sodium acetate. After adding 2.13 g (10 mmols) of freshly distilled bromopropiophenone, the reaction mixture is heated for 3 hours under reflux, whereupon the solution assumes a dark color. A solution of 2.61 g (11 mmols) of sodium m-nitrobenzenesulphonate and 4.4 g (110 mmols) of sodium hydroxide in a mixture of 20 ml of water and 8 ml of ethanol is then added and the mixture heated for a further 2 hours under reflux. The reaction mixture is cooled to room temperature and extracted with 5 portions of 100 ml of ether. The organic phases are washed with 3 portions of 50 ml of 2 N sodium hydroxide solution and 5 portions of 100 ml of water, combined and dried over anhydrous sodium sulphate. After filtering, and evaporating the filtrate, 1.4 g of crude product remain and this is purified by twice recrystallising from ethanol. Yield 0.7 g (25% of theory) of compound B. The thin layer chromatogram in

trichloromethane shows two minute traces of impurities alongside a main product. The infrared spectrum and the nuclear resonance spectrum are in agreement with the envisaged structure.

- 5 C. 5-Methoxy-6-chloro-2,3-dimethylquinoxaline  
2 g (10 mmols) of 4(7)-methoxy-5(6)-chlorobenzofuran are dissolved in 50 ml of ethyl acetate, mixed with 20 mg of platinum oxide and hydrogenated at room temperature under normal pressure. Over the course of 30 minutes, 900 ml of hydrogen are taken up, with the temperature rising to 49° C. After a further 90 minutes the temperature drops back to 25° C; the entire hydrogen uptake is 970 ml (99.5% of theory). The mixture is diluted with 20 ml of acetic acid ethyl ester, warmed to 40° C and filtered in a closed apparatus under nitrogen. The filtrate is mixed with 1.72 g (20 mmols) of diacetetyl and heated for 45 minutes under reflux. After cooling to room temperature, the mixture is evaporated to dryness and the residue (2.1 g) is recrystallised from water/methanol 1 : 1. Yield : 1.4 g; melting point: 83.5° to 85° C. Sublimation at 80° C and 0.04 mm Hg finally yields 1.3 g (59% of theory) of almost colourless crystals of the compound C.

The thin layer chromatogram with trichloromethane as the migrating agent shows a main zone and a slight impurity. The infrared spectrum and the nuclear resonance spectrum are in agreement with the expected structure.

- D. 6-Butoxy-2,3-dimethylquinoxaline  
1.6 g (9.2 mmols) of 6-hydroxy-2,3-dimethylquinoxaline, manufactured by ether scission of the 6-methoxy compound, 30 are dissolved in 15 ml of anhydrous dimethylformamide and mixed with 2.54 g (18.4 mmols) of potassium carbonate. After adding 1.47 g (10.8 mmols) of n-butyl bromide, the whole is kept for 30 minutes at 100° C internal temperature whilst stirring and excluding moisture. After slow cooling to 0° C, the 35 colorless crystals which have precipitated are filtered off and washed with a little water and then with a little ice-cold ethanol. Yield: 1.9 g of crude product which is purified by taking up in 5 ml of dimethylformamide and precipitating with 100 ml of water, so that 1.8 g (81% of theory) of compound D 40 are obtained.

It is possible to show by two-dimensional thin layer chromatography with cyclohexane-acetic acid ethyl ester, 6:4, that the compound suffers a certain decomposition at least in solution. The infrared spectrum and the nuclear resonance spectrum are in agreement with the envisaged structure.

- E. 5-Nitro-6-methoxy-2,3-dimethylquinoxaline  
18.55 g (100 mmols) of 6-methoxy-2,3-dimethylquinoxaline are introduced with stirring into 80 ml of 96% strength sulphuric acid, in the course of which the temperature rises to 50 70° C. After the solution has been cooled to 0° C, 15.7 g (125 mmols) of 50% strength nitric acid ("mixed acid") are added dropwise over the course of 15 minutes in such a way that the internal temperature does not exceed 5° C. Thereafter the 55 mixture is stirred for 4 hours at 0° – 5° C and is then poured onto 400 g of ice. The crude product which has precipitated is filtered off and suspended in excess 5% strength aqueous sodium carbonate. After renewed filtration and washing with water until neutral, 17.6 g of crude product are produced, 60 which are recrystallised from 280 ml of acetone and 350 ml of water. Yield : 12.75 g (56% of theory) of compound E.

The thin layer chromatogram in toluene/acetone, 9:1, shows a slight trace of impurity alongside a single product. The infrared spectrum shows the characteristic absorptions of 65 the functional groups; the nuclear resonance spectrum is in agreement with the envisaged structure.

- F. 5-Nitro-6-ethoxy-2,3-dimethylquinoxaline  
Starting from 6-ethoxy-2,3-dimethylquinoxaline, compound F is obtained in an analogous manner to that described in Instruction E, in a yield of 78 to 95% of theory.

The thin layer chromatogram in toluene/acetone, 9:1, shows slight impurities alongside the main product; the infrared spectrum and the nuclear resonance spectrum are in agreement with the structure.

- 75 G. 5-Amino-6-methoxy-2,3-dimethylquinoxaline

11.5 g (50 mmols) of 5-nitro-6-methoxy-2,3-dimethylquinoxaline, dissolved in 1,000 ml of ethanol, are mixed with Raney nickel (activity W 5) and hydrogenated at 65° C. 3.4 l of hydrogen (100% of theory) are taken up over the course of 2½ hours. After cooling to room temperature, the catalyst is filtered off and the filtrate is concentrated in vacuo, clarified by filtration with animal charcoal, and finally evaporated to dryness. Yield: 6.2 g (62% of theory) of compound G.

The thin layer chromatogram in toluene/acetone, 9:1, shows a slight impurity alongside the main product. The infrared spectrum and the nuclear resonance spectrum are in agreement with the structure of the desired compound.

#### H. 5-Amino-6-ethoxy-2,3-dimethylquinoxaline

5-Amino-6-ethoxy-2,3-dimethylquinoxaline (= compound H) is obtained in 65% yield from 5-nitro-6-ethoxy-2,3-dimethylquinoxaline in an analogous manner to that described in Instruction G.

The thin layer chromatogram in toluene/acetone, 9:1, shows a single product and the infrared spectrum and nuclear resonance spectrum correspond to the structure.

#### I. 2,3-Diphenylquinoxaline-6-carboxylic acid amide

3.26 g (10 mmols) of 2,3-diphenylquinoxaline-6-carboxylic acid are suspended in 30 ml of absolute benzene and mixed with 1 ml of dimethylformamide and 1.78 g (15 mmols) of thionyl chloride. On heating, the reaction mixture discolours at 60° C, with the acid slowly dissolving. After 8 hours the evolution of hydrochloric acid gas has ended. The excess thionyl chloride and about half the solvent are stripped in vacuo from the clear red-brown solution. The crystals which have precipitated are filtered off and washed with a little benzene. The infrared spectrum shows the bands which are characteristic for acid chlorides. After taking up in 50 ml of chloroform, adding 1 g of animal charcoal, filtering hot and evaporating the filtrate, 2.1 g (78% of theory) of yellowish-tinted crystals of melting point 168° to 169° C (decomposition) are obtained.

1 g (2.9 mmols) of the acid chloride thus obtained is heated for 1 hour under reflux with 20 ml of 24% strength ammonia. The colourless crystals which have precipitated after cooling are filtered off, washed with a little cold water and dried in vacuo. Yield: 0.9 g (96% of theory). recrystallisation from acetic acid ethyl ester/methanol, 1:1, finally yields fine colourless needles of the compound I, the infrared spectrum of which is in agreement with the envisaged structure. The thin layer chromatogram in chloroform/butyl acetate, 7:3, shows two slight impurities alongside the main zone.

#### J. 2,3-Diphenylquinoxaline-6-carboxylic acid methyl ester

950 mg (2.75 mmols) of the acid chloride as described in Instruction I are heated for 15 minutes in 15 ml of methanol under reflux, whereupon the colour changes to lemon yellow and a yellow precipitate begins to separate out. After slow cooling the product is filtered off, washed with a little icecold methanol and dried in vacuo. The 600 mg of ester thus obtained are recrystallised from 40 ml of methanol. Yield: 500 mg (54% of theory) of colourless platelets of the compound J.

The infrared spectrum and the nuclear resonance spectrum show the bands to be expected for the envisaged structure.

#### K. 2,3-Dimethylquinoxaline-6-carboxylic acid amide

2.02 g (10 mmols) of 2,3-dimethylquinoxaline-6-carboxylic acid are dissolved in 200 ml of 1,2-dimethoxyethane. After adding 1.01 g (10 mmols) of triethylamine, the mixture is cooled to 0° C. 1.2 g (11 mmols) of chloroformic acid ethyl ester are added dropwise with vigorous stirring in such a way that the internal temperature does not exceed 10° C. The mixture is stirred for a further 3 hours at room temperature. After completion of the reaction, 20 ml of 24% strength ammonia are added and the mixture is warmed to 60° C for 1 hour. After evaporation under reduced pressure and recrystallization from methanol, 1.3 g (65% of theory) of colourless crystals of the compound K are obtained. The thin layer chromatogram with propanol/24% strength ammonia, 8:2, as the migrating agent shows a single substance. The infrared spectrum and the nuclear resonance spectrum are in agreement with the postulated structure.

#### L. 5-Benzoylaminio-6-methoxy-2,3-dimethylquinoxaline

1.0 g (5 mmols) of compound G is dissolved in 15 ml of dimethylformamide and mixed with 1.2 g (12 mmols) of triethylamine. After cooling to 0° C, the solution thus obtained is mixed with 1.7 g (12 mmols) of benzoyl chloride whilst stirring. Stirring is continued for 2 hours at 0° C and the reaction mixture is then poured out onto 200 g of ice-water mixture. The colorless precipitate which thereupon forms is filtered off and washed with cold water. After recrystallization from methanol, 0.7 g (50% of theory) of the compound L are obtained.

The thin layer chromatogram with toluene : acetone, 9:1, as the migrating agent shows a main zone. The infrared spectrum and nuclear resonance spectrum are in agreement with the postulated structure.

The compounds M to RR of Table I are manufactured analogously to the compounds A to L.

TABLE I

| Compound | Residues in Formula (1) |                 |                                  |                                      | Melting point, °C. | Analysis, percent |      |       |       |      |       |
|----------|-------------------------|-----------------|----------------------------------|--------------------------------------|--------------------|-------------------|------|-------|-------|------|-------|
|          | A <sub>1</sub>          | A <sub>2</sub>  | D                                | E                                    |                    | C                 | H    | N     | C     | H    | N     |
| A        | CH <sub>3</sub>         | CH <sub>3</sub> | 6-OC <sub>2</sub> H <sub>5</sub> | H                                    | 108.9              | 71.26             | 6.98 | 13.85 | 71.33 | 7.00 | 13.97 |
| B        | CH <sub>3</sub>         | CH <sub>5</sub> | 6-OCH <sub>3</sub>               | 7-OCH <sub>3</sub>                   | 160.4              | 72.84             | 5.75 | 9.99  | 72.73 | 5.83 | 9.94  |
| C        | CH <sub>3</sub>         | CH <sub>3</sub> | 5-OCH <sub>3</sub>               | 6-Cl                                 | 91.1               | 59.33             | 4.97 | 12.58 | 59.30 | 4.97 | 12.59 |
| D        | CH <sub>3</sub>         | CH <sub>3</sub> | 6-OC <sub>2</sub> H <sub>5</sub> | H                                    | 50.4               | 73.01             | 7.88 | 12.17 | 73.16 | 7.86 | 12.34 |
| E        | CH <sub>3</sub>         | CH <sub>3</sub> | 6-OCH <sub>3</sub>               | 5-NO <sub>2</sub>                    | 160.1              | 56.65             | 4.75 | 18.02 | 56.68 | 4.80 | 18.04 |
| F        | CH <sub>3</sub>         | CH <sub>3</sub> | 6-OC <sub>2</sub> H <sub>5</sub> | 5-NO <sub>2</sub>                    | 144.2              | 58.29             | 5.30 | 17.00 | 58.28 | 5.34 | 17.00 |
| G        | CH <sub>3</sub>         | CH <sub>3</sub> | 6-OCH <sub>3</sub>               | 5-NH <sub>2</sub>                    | 135.7              | 65.00             | 6.45 | 20.68 | 65.09 | 6.49 | 20.68 |
| H        | CH <sub>3</sub>         | CH <sub>3</sub> | 6-OC <sub>2</sub> H <sub>5</sub> | 5-NH <sub>2</sub>                    | 138.0              | 66.34             | 6.96 | 19.34 | 66.47 | 6.91 | 19.17 |
| I        | CH <sub>5</sub>         | CH <sub>5</sub> | 6-CO NH <sub>2</sub>             | H                                    | 254.2              | 77.52             | 4.65 | 12.92 | 77.48 | 4.54 | 12.98 |
| J        | CH <sub>5</sub>         | CH <sub>5</sub> | 6-COOCH <sub>3</sub>             | H                                    | 145.2              | 77.63             | 4.74 | 8.23  | 77.72 | 4.65 | 8.23  |
| K        | CH <sub>3</sub>         | CH <sub>3</sub> | 6-CONH <sub>2</sub>              | H                                    | 1250               | 65.67             | 5.50 | 20.80 | 65.18 | 5.63 | 20.65 |
| L        | CH <sub>3</sub>         | CH <sub>3</sub> | 6-OCH <sub>3</sub>               | 5-NH-COC <sub>2</sub> H <sub>5</sub> | 196.3              | 70.34             | 5.57 | 13.67 | 70.49 | 5.44 | 13.92 |
| M        | CH <sub>5</sub>         | CH <sub>5</sub> | 5-OCH <sub>3</sub>               | H                                    | 192.2              | 80.75             | 5.16 | 8.97  | 80.66 | 5.15 | 8.98  |
| N        | CH <sub>5</sub>         | CH <sub>5</sub> | 6-OC <sub>2</sub> H <sub>5</sub> | H                                    | 144.0              | 81.33             | 6.26 | 7.90  | 81.94 | 6.32 | 7.91  |
| O        | CH <sub>3</sub>         | CH <sub>3</sub> | 6-OCH <sub>3</sub>               | H                                    | 100.3              | 70.19             | 6.47 | 14.88 | 69.88 | 6.47 | 15.29 |
| P        | CH <sub>5</sub>         | CH <sub>5</sub> | 6-OCH <sub>3</sub>               | H                                    | 160.8              | 80.75             | 5.16 | 8.97  | 80.48 | 5.25 | 9.01  |
| Q        | CH <sub>3</sub>         | CH <sub>5</sub> | 6-OCH <sub>3</sub>               | H                                    | 122.0              | 76.78             | 5.64 | 11.19 | 76.41 | 5.70 | 11.25 |
| R        | CH <sub>5</sub>         | CH <sub>5</sub> | 6-OCH <sub>3</sub>               | H                                    | 88.6               | 76.78             | 5.64 | 11.19 | 76.41 | 5.70 | 11.25 |
| S        | CH <sub>5</sub>         | CH <sub>5</sub> | 6-OC <sub>2</sub> H <sub>5</sub> | H                                    | 154.3              | 80.88             | 5.56 | 8.58  | 81.15 | 5.51 | 8.60  |
| T        | CH <sub>3</sub>         | CH <sub>3</sub> | 6-COOH                           | H                                    | 262.6              | 65.34             | 4.98 | 13.85 | 65.31 | 4.94 | 13.88 |
| U        | CH <sub>5</sub>         | CH <sub>5</sub> | 6-COOH                           | H                                    | 290.3              | 77.29             | 4.32 | 8.58  | 77.11 | 4.22 | 8.68  |
| V        | CH <sub>3</sub>         | CH <sub>3</sub> | 6-COOCH <sub>3</sub>             | H                                    | 91.6               | 66.65             | 5.59 | 12.96 | 66.70 | 5.55 | 12.96 |
| W        | CH <sub>5</sub>         | CH <sub>5</sub> | 5-OCH <sub>3</sub>               | 6-Cl                                 | 140.0              | 72.73             | 4.36 | 8.08  | 72.47 | 4.46 | 8.10  |
| X        | CH <sub>3</sub>         | CH <sub>3</sub> | 6-OCH <sub>3</sub>               | 5-Cl                                 | 147.3              | 59.33             | 4.98 | 12.58 | 59.24 | 4.98 | 12.56 |
| Y        | CH <sub>5</sub>         | CH <sub>5</sub> | 5-OCH <sub>3</sub>               | 5-Cl                                 | 186.4              | 72.73             | 4.36 | 8.08  | 72.39 | 4.33 | 8.12  |
| Z        | CH <sub>3</sub>         | CH <sub>3</sub> | 5-OCH <sub>3</sub>               | 8-OCH <sub>3</sub>                   | 171.4              | 66.04             | 6.46 | 12.84 | 66.09 | 6.42 | 12.93 |
| AA       | CH <sub>5</sub>         | CH <sub>5</sub> | 5-OCH <sub>3</sub>               | 8-OCH <sub>3</sub>                   | 232.2              | 77.17             | 5.30 | 8.18  | 77.08 | 5.35 | 8.22  |
| BB       | CH <sub>3</sub>         | CH <sub>3</sub> | 6-OCH <sub>3</sub>               | 7-OCH <sub>3</sub>                   | 178.1              | 66.04             | 6.46 | 12.83 | 65.97 | 6.49 | 12.86 |
| CC       | CH <sub>5</sub>         | CH <sub>5</sub> | 6-OCH <sub>3</sub>               | 7-OCH <sub>3</sub>                   | 252.4              | 77.17             | 5.30 | 8.18  | 77.10 | 5.26 | 8.16  |
| DD       | CH <sub>3</sub>         | CH <sub>3</sub> | 5-OCH <sub>3</sub>               | H                                    | 119.1              | 70.19             | 6.43 | 14.88 | 70.23 | 6.44 | 14.93 |
| EE       | CH <sub>3</sub>         | CH <sub>3</sub> | 6-OCH <sub>3</sub>               | 5-NH-COCH <sub>3</sub>               | 183.9              | 63.66             | 6.16 | 17.13 | 63.67 | 6.58 | 17.23 |
| FF       | CH <sub>5</sub>         | CH <sub>5</sub> | 5-OCH <sub>3</sub>               | 8-NHCOCH <sub>3</sub>                | 238.9              | 74.78             | 5.18 | 11.37 | 74.99 | 5.15 | 11.24 |
| GG       | CH <sub>3</sub>         | CH <sub>3</sub> | 5-OCH <sub>3</sub>               | 8-NHCOCH <sub>3</sub>                | 234.7              | 63.66             | 6.16 | 17.13 | 63.52 | 6.19 | 17.19 |

Table I—Continued

| Compound | Residues in Formula (1)       |                               |                                                       |                     | Melting point, °C. | Analysis, percent |      |       |
|----------|-------------------------------|-------------------------------|-------------------------------------------------------|---------------------|--------------------|-------------------|------|-------|
|          | A <sub>1</sub>                | A <sub>2</sub>                | D                                                     | E                   |                    | C                 | H    | N     |
| HH.....  | C <sub>6</sub> H <sub>5</sub> | C <sub>6</sub> H <sub>5</sub> | 6-COOOC <sub>2</sub> H <sub>5</sub>                   | H                   | 151.9              | 77.95             | 5.12 | 7.90  |
| II.....  | CH <sub>3</sub>               | CH <sub>3</sub>               | 6-COOOC <sub>2</sub> H <sub>5</sub>                   | H                   | 100.6              | 67.81             | 6.13 | 12.16 |
| JJ.....  | CH <sub>3</sub>               | CH <sub>3</sub>               | 6-CN                                                  | H                   | 205.9              | 72.11             | 4.95 | 22.94 |
| KK.....  | C <sub>6</sub> H <sub>5</sub> | C <sub>6</sub> H <sub>5</sub> | 6-CN                                                  | H                   | 181.4              | 82.06             | 4.26 | 13.67 |
| LL.....  | CH <sub>3</sub>               | CH <sub>3</sub>               | 6-CO(N(C <sub>2</sub> H <sub>5</sub> ) <sub>2</sub> ) | H                   | 73.3               | 70.01             | 7.44 | 16.33 |
| MM.....  | C <sub>6</sub> H <sub>5</sub> | C <sub>6</sub> H <sub>5</sub> | 6-CO(N(C <sub>2</sub> H <sub>5</sub> ) <sub>2</sub> ) | H                   | 137.0              | 78.71             | 6.08 | 11.05 |
| NN.....  | CH <sub>3</sub>               | CH <sub>3</sub>               | 6-OCH <sub>3</sub>                                    | 7-NH <sub>2</sub>   | 1252               | 65.01             | 5.09 | 20.68 |
| PP.....  | CH <sub>3</sub>               | CH <sub>3</sub>               | 5-OCH <sub>3</sub>                                    | 8-NHCH <sub>3</sub> | 151.1              | 66.34             | 6.96 | 19.34 |
| QQ.....  | CH <sub>3</sub>               | CH <sub>3</sub>               | 5-OCH <sub>3</sub>                                    | 8-CH <sub>3</sub>   | 124.4              | 71.26             | 6.98 | 13.85 |
| RR.....  | C <sub>6</sub> H <sub>5</sub> | C <sub>6</sub> H <sub>5</sub> | 5-OCH <sub>3</sub>                                    | 8-CH <sub>3</sub>   | 190.7              | 80.96             | 5.56 | 8.58  |
|          |                               |                               |                                                       |                     |                    | 81.04             | 7.04 | 13.91 |
|          |                               |                               |                                                       |                     |                    |                   | 5.60 | 8.54  |

<sup>1</sup> Decomposition.

## EXAMPLE 1

A solution consisting of 3.3 ml of 6% strength gelatine, 2.0 ml of a 1% ml solution of the hardener 2,4-dichloro-6-phenylamino-1,3,5-triazine-3'-sulphonic acid, 0.5 ml of a 2.10<sup>-3</sup> 20 molar solution of compound U in dimethylformamide and 4.2 ml of water is cast on a glass plate of size 13 cm × 18 cm. After drying, a solution consisting of 3.3 ml of 6% strength gelating, 3.3 ml of a silver bromide emulsion, containing 5.3 g of silver per 100 g of emulsion, 2.0 ml of the above hardener, 0.3 ml of 25 a 1% strength solution of the blue-green dyestuff of formula

7.2 minutes soaking

8.4 minutes fixing as under 2.)

9. 10 minutes soaking.

After drying, the image which has been cleanly bleached colourless is obtained with a distinct stepped gradation of the wedge used as the original.

## EXAMPLE 2

If, instead of compound U, the compound I is employed and

(1.1)



and 1.1 ml of water is cast on top. After drying of the combined layer thus obtained, a step wedge is copied onto it (50. 50 LUX, 3 sec.). Thereafter the copy is developed in accordance with the following instruction:

1. 6 minutes development in a bath which per liter contains 50 g of anhydrous sodium sulphite, 0.2 g of 1-phenyl-3-pyrazolidone, 6 g of hydroquinone, 35 g of anhydrous sodium carbonate, 4 g of potassium bromide and 0.3 g of benztriazole

2. 2 minutes fixing with a solution of 200 g of sodium thiosulphate, 10 g of anhydrous sodium sulphite, 20 g of sodium acetate and 10 ml of glacial acetic acid per liter of water

3. 4 minutes soaking

4. 6 minutes dyestuff bleaching with a solution of 10 g of potassium iodide in 1 l of 1 N sulphuric acid

5. 2 minutes soaking

the procedure described in Example 1 is followed, a clean positive image of the exposed wedge is again obtained. If, instead of compound U, compound KK is employed as an acetone solution and the procedure of Example 1 is followed, a clean positive image of the wedge used as an original is again obtained.

The compound U can with equal success be replaced by the compound L, which is applied as an alcoholic solution.

## EXAMPLE 3

55 A photographic material with three color layers contains, on an opaque white cellulose acetate film, a red-sensitive silver bromide emulsion with the blue-green dyestuff of formula



6. 2 minutes bleaching of the residual silver with a bath containing 150 ml of 37% strength hydrochloric acid, 25 g of copper sulphate and 30 g of potassium bromide per liter

on top of this an empty gelatine separating layer, then a green-sensitive silver bromide emulsion with the purple dye-stuff of formula

13



14



After a further separating layer, there follows a layer with a yellow filter dyestuff or with colloidal silver acting as a yellow filter. On top of this there is a silver bromide layer with the yellow dyestuff of formula

(2.3)



and a covering layer. All layers are hardened with a halogenotriazine compound such as 2,4-dichloro-6-phenylamino-1,3,5-triazine-3'-sulphonic acid.

This copying material is successively exposed under a step wedge in the three spectral regions blue (Wratten filter Kodak 2 B + 49), green (Wratten filter Kodak 16 + 61) and red (Wratten filter Kodak 2 x 29), and developed for 7 minutes, and fixed, as described in Example 1. Thereafter bleaching is carried out in a silver dyestuff bleaching bath which per liter contains 27 ml of 96% strength sulphuric acid, 10 g of potassium iodide and 10 ml of a  $4 \cdot 10^{-2}$  molar solution of the compound DD in ethanol. After a brief soaking, the residual silver is oxidised as described in Example 1 under 6.), and the material is soaked and fixed as described above. After thorough rinsing and after drying, a grey wedge bleached to white is obtained, the gradation of which corresponds to the original.

#### EXAMPLE 4

Instead of the compound DD as in Example 3, the compound Z or another of the quinoxalines quoted in Table I, dissolved in a suitable photographically inactive water-miscible solvent, can be employed. If the same procedure as in Example 3 is then followed, then on suitable matching the grey image of the original used, bleached cleanly to white in the appropriate areas, is again obtained.

#### EXAMPLE 5

A photographic material as described in Example 3 is exposed in the three spectral ranges as indicated. Thereafter the copy is developed as follows:

1. 7 minutes development in a bath which per litre contains 50 g of anhydrous sodium sulphite, 0.2 g of 1-phenyl-3-pyrazolidone, 6 g of hydroquinone, 35 g of anhydrous sodium carbonate, 4 g of potassium bromide, 0.3 g of benztriazole and 20 ml of a  $4 \cdot 10^{-2}$  molar solution of compound U in dimethyl-formamide
2. 2 minutes fixing with a solution of 200 g of sodium thiosulphate, 10 g of anhydrous sodium sulphite and 10 ml of glacial acetic acid per liter
3. 2 minutes soaking
4. 10 minutes dyestuff bleaching with a solution of 10 g of potassium iodide in 1 litre of sulphuric acid
5. 2 minutes soaking
6. 8 minutes bleaching of the residual silver with a bath which contains 150 ml of 37% strength hydrochloric acid, 25 g of copper sulphate and 30 g of potassium bromide per liter
7. 2 minutes soaking
8. 3 minutes fixing as under 2.)
9. 10 minutes soaking.

10 After drying, a grey wedge with clean whites and distinctly stepped gradation is obtained.

Instead of the compound U, the compound T or the compound JJ can be used with equal success.



#### EXAMPLE 6

25 A solution of the following composition is cast onto a glass plate of size 13 cm x 18 cm: 3.3 ml of 6% strength gelatine, 3.3 ml of a silver bromide emulsion which contains 5.3 g of silver per 100 g of emulsion, 1.0 ml of a 1% strength solution of the hardener described in Example 1, 0.3 ml of a 1% strength solution of the blue-green dyestuff of formula

1.1 and 2.1 ml of water.

After drying, a step wedge is copied onto the layer thus obtained, and the plate is then treated according to the following instruction:

1. 10 minutes development in a bath which per liter contains 20 g of anhydrous sodium sulphite, 1 g of 4-methylaminophenol sulphate, 4 g of hydroquinone, 10 g of anhydrous sodium carbonate, 2 g of potassium bromide and 3 g of sodium thiocyanate;
2. 2 minutes soaking;
3. 2 minutes oxidising with a solution of 5 g of potassium bichromate and 5 ml of 96% strength sulphuric acid per liter of solution;
4. 4 minutes soaking;
5. 5 minutes washing with a solution of 50 g of anhydrous sodium sulphite per liter;
6. 3 minutes soaking;
7. 4 minutes development with a solution consisting of 2 g of Calgon, 50 g of anhydrous sodium sulphite, 10 g of hydroquinone, 50 g of anhydrous sodium carbonate, 2 g of 1-phenyl-3-pyrazolidone and 20 ml of a 1% strength t-butyl-aminoborane per liter;
8. 2 minutes soaking;
9. 6 minutes dyestuff bleaching with a colour bleaching bath which per litre contains 27 ml of 96% strength sulphuric acid, 10 g of potassium iodide and 10 ml of a  $4 \cdot 10^{-2}$  molar solution of the compound H in ethanol;
10. 2 minutes soaking;
11. 2 minutes bleaching of the residual silver as described in Example 1 under 6.);
12. 2 minutes soaking;
13. 4 minutes fixing as described in Example 1 under 2.);
14. 10 minutes soaking.

After drying, an image of the wedge used, cleanly bleached to colourless, with contrary gradation, is obtained.

Instead of the compound H, it is possible to use the compound PP or another of the quinoxalines described in the table, in a suitable photographically inactive water-miscible solvent. If the procedure described in this example is then followed, an image of the exposed wedge, cleanly bleached to colourless, with contrary gradation, is again obtained.

#### EXAMPLE 7

75 A solution consisting of 3.3 ml of 6% strength gelatine, 3.3 ml of a silver bromide emulsion containing 5.3 g of silver per

100 g of emulsion, 1.0 ml of a 1% strength solution of the cur-  
ing agent described in Example 1, 0.3 ml of a 1% strength  
solution of the blue-green dyestuff of formula 1.1 described in  
Example 1, 0.5 ml of a  $4 \times 10^{-2}$  molar solution of the com-  
pound U in dimethylformamide and 1.6 ml of water is cast on  
a glass plate of size 13 cm  $\times$  18 cm. After drying, a step wedge  
is copied onto the layer thus obtained (50 LUX, 10 sec.) and  
the copy is processed as described in Example 1.

After drying, a positive image, cleanly bleached to colorless,  
of the wedge used as the original is obtained.

The compound U can be replaced by the compound EE,  
dissolved in methanol. If then the procedure described in this  
example is followed, a positive image, cleanly bleached to  
colourless, of the original used is again obtained.

Instead of the compound U, it is possible with equally good  
success to use the quinoxaline II from the table, as an alcoholic  
solution.

#### EXAMPLE 8

A photographic material as described in Example 3 is ex-  
posed in the three spectral ranges as indicated in Example 3.  
The copy is then treated as follows:

1. 7 minutes development with a bath which per liter con-  
tains 20 g of anhydrous sodium sulphite, 10 g of an-  
hydrous sodium carbonate, 4 g of hydroquinone, 1 g of 4-  
methylaminophenol sulphate, 2 g of potassium bromide  
and 10 ml of a  $4 \times 10^{-2}$  molar solution of the compound U  
in dimethylformamide;
2. 2 minutes fixing with a solution of 200 g of sodium  
thiosulphate, 15 g of anhydrous sodium sulphite, 25 g of  
crystallized sodium acetate and 13 ml of glacial acetic  
acid per liter;
3. 2 minutes soaking;
4. 10 minutes dyestuff bleaching using a composition which  
per liter contains 10 g of potassium iodide, 27 ml of 96%  
strength sulphuric acid and 5 ml of a  $4 \times 10^{-2}$  molar solution  
of the compound U in dimethylformamide;
5. 2 minutes soaking;
6. 8 minutes bleaching of the residual silver as described in  
Example 5 under 6);
7. 2 minutes soaking;
8. 3 minutes fixing as under 2.); and
9. 10 minutes soaking.

After drying, a positive image, cleanly bleached to white, of  
the original used is obtained.

#### EXAMPLE 9

A solution consisting of 3.3 ml of 6% strength gelatine, 2.0  
ml of a 1% strength solution of the hardener described in Ex-  
ample 1, 3.3 ml of a silver bromide emulsion which contains  
5.3 g of silver per 100 g of emulsion, 0.3 ml of a 1% strength  
solution of the blue-green dyestuff of formula (1.1) and 1.1 ml  
of water is cast onto a glass plate of size 13 cm  $\times$  18 cm. After  
drying, a step wedge is copied onto it (50 Lux, 3 seconds) and  
the copy is treated as follows:

6 minutes dyestuff bleaching with a solution which per liter  
contains 27 ml of 96% strength sulphuric acid, 10 g of potas-  
sium iodide, and in each case 10 ml of a  $4 \times 10^{-2}$  molar solution  
of one of the compounds BB, V, R, O, I, E, NN, II or QQ in  
ethanol or another suitable water-miscible photographically  
inactive solvent.

After 2 minutes soaking the residual silver is oxidised as  
described in Example 1 under 6) and the material is soaked  
and fixed as described above. The copy is thoroughly washed  
and dried. In each case a blue-green wedge, cleanly bleached  
to colourless, of which the gradation corresponds to that of  
the original, is obtained.

#### EXAMPLE 10

A solution consisting of 3.3 ml of gelatine, 1.0 ml of a 1%  
strength solution of the purple dyestuff of formula

5



10

2.0 ml of a 1% strength solution of the hardener described in  
Example 1, 3.3 ml of a silver bromide emulsion containing 5.3  
g of silver per 100 g of emulsion and 0.4 ml of water, is cast  
onto a glass plate of size 13 cm  $\times$  18 cm. After drying, a step  
wedge is copied thereon (50 Lux, 5 seconds) and the copy is  
treated as follows:

Developing and fixing as described in Example 1. 6 minutes  
dyestuff bleaching with a solution which per liter contains 10 g  
of potassium iodide, 27 ml of 96% strength sulphuric acid and  
in each case 10 ml of a  $4 \times 10^{-2}$  molar solution of the com-  
pound X, Q, G, B or F in ethanol or another suitable water-  
miscible photographically inactive solvent. After a brief soaking,  
the residual silver is oxidised as described above, and the  
material is soaked and fixed. After thorough rinsing and dry-  
ing, an image, cleanly bleached to colorless, with a distinctly  
stepped gradation of the original used is thus obtained in all  
cases.

#### EXAMPLE 11

A glass plate of size 13 cm  $\times$  18 cm is coated with a solution  
which contains 3.3 ml of 6% strength gelatine, 2.0 ml of a 1%  
strength solution of the hardener described in Example 1, 3.3  
ml of a silver bromide emulsion containing 5.3 g of silver per  
100 g of emulsion, 0.5 ml of the yellow dyestuff of formula

30



40

and 0.9 ml of water. After drying, a step wedge is copied  
thereon (50 Lux, 5 seconds) and the material is treated  
analogously to Examples 9 and 10, with the colour bleaching  
bath, instead of containing the compounds mentioned there,  
containing 10 ml of a  $4 \times 10^{-2}$  molar solution of one of the  
substances C, D, P, CC, JJ, LL or GG in methanol or another  
suitable water-miscible photographically inactive solvent.  
After drying, a yellow image of the original used, cleanly  
bleached to colorless, with the gradation corresponding to  
that of the original, is then obtained.

55

We claim:

1. Process for the manufacture of color photographic  
images according to the silver dyestuff bleaching process on a  
light-sensitive photographic material which on a substrate  
contains at least one silver halide emulsion layer with a  
dyestuff which can be bleached image-wise, by exposure,  
development of the silver image and dyestuff bleaching, which  
comprises dyestuff bleaching in the presence of a quinoxaline  
of the formula

65



70

as dyestuff bleaching catalyst, in which A<sub>1</sub> and A<sub>2</sub> each is an  
alkyl radical with at most 5 carbon atoms or a phenyl radical,  
D is a radical of the formula -CN, -O-R, -COO-R<sub>1</sub> or



in which R is an alkyl radical with at most five carbon atoms and R<sub>1</sub> and R<sub>2</sub> each is a hydrogen atom or an alkyl radical with at most five carbon atoms, and E is a hydrogen or halogen atom, an alkyl or alkoxy group with at most five carbon atoms, a nitro group, an unsubstituted amino group, an alkylamino group with at most four carbon atoms or an acylamino group.

2. Process according to claim 1, which comprises using a quinoxaline of the formula



as a dyestuff bleaching catalyst, in which A<sub>1</sub> and A<sub>2</sub> each is a methyl or phenyl radical, and D is a radical of the formula —O—R, —COO—R<sub>1</sub> or



3. Process according to claim 1, which comprises using a quinoxaline of the formula



as a dyestuff bleaching catalyst, in which D is an alkoxy group with one to four carbon atoms and E is a hydrogen atom, a halogen atom, an alkyl or alkoxy group with at most five carbon atoms, a nitro, amino or alkylamino group with at most 4 carbon atoms or an acylamino group, and A<sub>1</sub> and A<sub>2</sub> each is a methyl or phenyl radical.

4. Process according to claim 1, which comprises using a quinoxaline of the formula



as a dyestuff bleaching catalyst, in which D is a methoxy or ethoxy group, E is a chlorine atom, a methyl, methoxy, nitro,

amino, methylamino or acylamino group, in which acyl is the radical of an alkanecarboxylic acid with one to five carbon atoms, benzoic acid, and benzoic acid substituted by halogen, alkyl, nitro, alkoxy, hydroxy or amino and A<sub>1</sub> and A<sub>2</sub> each is a methyl or phenyl radical.

5. Process according to claim 3, which comprises using a quinoxaline of the formula



10 15 as a dyestuff bleaching catalyst, in which D is a methoxy or ethoxy group and E is a methoxy, methylamino or amino group.

6. Process according to claim 2, in which A<sub>1</sub> is methyl.

7. Process according to claim 6, in which A<sub>2</sub> is methyl.

20 8. Process according to claim 5, in which A<sub>1</sub> and A<sub>2</sub> is each methyl.

9. Process according to claim 5, in which D is methoxy and A<sub>1</sub> is methyl.

10. Process according to claim 9, in which A<sub>2</sub> is methyl.

25 11. Process according to claim 1, which comprises using a quinoxaline of the formula



30 as a dyestuff bleaching catalyst, in which D is a radical of the formula —CN, —COOR<sub>1</sub> or

35



in which R<sub>1</sub> and R<sub>2</sub> each is an alkyl radical with at most five carbon atoms or a hydrogen atom and A<sub>1</sub> and A<sub>2</sub> each is an alkyl radical with at most five carbon atoms or a phenyl radical.

45 12. Process according to claim 11, in which A<sub>1</sub> and A<sub>2</sub> each is a methyl or phenyl radical.

13. Process according to claim 12, in which D is a radical of the formula —COOR<sub>1</sub>, in which R<sub>1</sub> is an alkyl radical with at most five carbon atoms or a hydrogen atom, and A<sub>1</sub> is methyl.

50 14. Process according to claim 13, in which A<sub>1</sub> and A<sub>2</sub> is each methyl and R<sub>1</sub> is hydrogen.

15. Photographic light-sensitive material for the silver dyestuff bleaching process, which contains a quinoxaline of the composition indicated in claim 1 as a dyestuff bleaching catalyst in at least one layer on a support.

55 16. A photographic processing bath for silver dyestuff bleaching material, which contains at least a quinoxaline of the composition indicated in claim 1 as a dyestuff bleaching catalyst.

\* \* \* \* \*